

## 1

2,740,711

### IRON CHROMIUM MOLYBDENUM TITANIUM BASE ALLOY

Schuylerville A. Herres and Thomas K. Redden, Albany, N. Y., assignors to Allegheny Ludlum Steel Corporation, Brackenridge, Pa., a corporation of Pennsylvania

No Drawing. Application April 29, 1952,  
Serial No. 285,078

4 Claims. (Cl. 75—175.5)

This invention relates to a new and improved titanium base alloy having ternary metal alloying additions of iron, chromium and molybdenum, and wherein oxygen and nitrogen are maintained within maximum limits.

This application is a continuation-in-part of our co-pending application No. 118,723 of September 29, 1949 entitled "Titanium Alloys."

It has been an object of our present invention to produce a relatively inexpensive titanium alloy having a stabilized all beta phase structure;

Another object is to provide an improved titanium base alloy which may make use of ferro alloys as additional agents in the melt;

A further object has been to produce titanium base alloys which are substantially free of intermetallic compounds and their resultant harmful effects;

These and many other objects of our invention will appear to those skilled in the art from the following description.

The alloying content of our alloy is critical and particularly, from the standpoint of a retained beta body-centered cubic form of lattice structure which is characteristic of titanium metal when heated above about 1625° F. The alloy here being considered saves scarce and strategic elements and is suitable for structural purposes, such as in airplanes, where the service temperature does not go above about 400° F. and a good ductility is needed with a high tensile strength.

Unalloyed titanium normally exists in a hexagonal, closely-packed, crystalline structure at room temperature and transforms on heating to above about 1625° F. to a body-centered cubic lattice crystalline structure. The present invention deals with alloying additions stabilizing and completely retaining the high temperature beta structure of titanium, so that it is fully available at room temperature without the presence of alpha phase titanium. In this manner, we have been able to produce an alloy having an excellent ductility with a good tensile strength, impact, and other properties.

Reheating an alloy of the present invention within a range of about 500° to 1100° F. after its solution heat treatment will result in a decomposition of the retained beta phase, a resultant precipitation of the alpha phase, and serious loss of ductility. The alloy is, however, very useful in service at room temperature up to about 400° F. due to its combination of high strength and good ductility. Also, it is capable of being cold worked and annealed, thus facilitating the processing of sheet and strip products.

## 2

In carrying out our invention, we employ a titanium base alloy of the following composition:

Table I

| General Range             | Optimum Range             |
|---------------------------|---------------------------|
| Mo=1.5 to 10%             | Mo=2.5 to 6.5%            |
| Cr=1.5 to 11%             | Cr=2.5 to 6.5%            |
| Fe=3.0 to 8%              | Fe=3.5 to 6.0%            |
| O <sub>2</sub> =.20% max. | O <sub>2</sub> =.20% max. |
| N <sub>2</sub> =.10% max. | N <sub>2</sub> =.10% max. |

In the above alloys, the remainder is titanium with incidental impurities or substantially all titanium and the alloying element contents are critical in their specified ranges. The metal alloying elements are also critical in their total content (molybdenum + iron + chromium) in that such total should be above about 11.00% and below about 20%; the optimum range being about 13 to 16%.

We have found that the three metal elements in combination all tend to stabilize the beta phase of titanium. Further, the use of these metal elements within the ranges specified produces an alloy which is more stable than one made from one of the elements alone and produces an alloy that is free from the harmful effects due to the presence of intermetallic compounds that are present in binary iron-titanium and chromium-titanium alloying systems. The metal alloying elements, as an optimum, are introduced at one time to the melt and as ferro alloy-additions. The latter type of additions are more readily soluble in the melt and are less scarce and strategic than the single elements, themselves. The total content of the metal alloying elements is highly critical and particularly so from the standpoint of the retention of the beta phase of titanium.

Heat treatment consists of a solution treatment in the range of about 1200° to 1500° F., followed by air cooling. This treatment provides an all beta-phase structure having the required ductility and tensile properties. The alloys may be hot worked within a range of about 1200 to 1700° F. and may also be cold worked at room temperature to produce a resultant increase of tensile strength and decrease in ductility. Titanium of commercial purity may be used in making the alloys, but it is important to maintain the oxygen and nitrogen gaseous alloying elements within the previously specified maximum amounts to obtain requisite properties.

The following is indicative of the properties of alloys of our alloy invention after they have been solution treated in the manner previously explained. Melt No. K669 which has a total metal alloying content of 11%, illustrates the importance of the lower critical total metal alloying content. Melt K662 which has a molybdenum content that is well below the critical minimum of 1.5% required and is thus not an alloy of our invention, illus-

3  
trates the importance of the individual contents of the metal alloying elements:

amount up to about .10% maximum, about 1.5 to 10% molybdenum, about 1.5 to 11% chromium, about 3 to

Table II

| Heat No. | Composition           |               |                              |             |             | Tensile Strength, lbs./sq. in. | El., Percent | R. A., Percent | Ingot Hardness, BHN |  |  |  |  |
|----------|-----------------------|---------------|------------------------------|-------------|-------------|--------------------------------|--------------|----------------|---------------------|--|--|--|--|
|          | Using Ferro Additions |               | Based On Individual Elements |             |             |                                |              |                |                     |  |  |  |  |
|          | FeCr, Percent         | FeMo, Percent | Fe, Percent                  | Cr, Percent | Mo, Percent |                                |              |                |                     |  |  |  |  |
| K642     | 10                    | 10            | 6.7                          | 7.0         | 6.3         | 173,000                        | 11           | 19             | 332                 |  |  |  |  |
| K645     | 9                     | 3             | 3.8                          | 6.3         | 1.9         | 167,000                        | 1            | 1.6            | 332                 |  |  |  |  |
| K662     | 10                    | 2             | 3.75                         | 7.0         | 1.25        | 167,000                        | 19           | 48.7           | 311                 |  |  |  |  |
| K663     | 2                     | 10            | 4.25                         | 1.4         | 6.35        | 156,000                        | 12           | 48             | 321                 |  |  |  |  |
| K664     | 4                     | 8             | 4.15                         | 2.8         | 5.05        | 158,500                        | 14           | 47             | 305                 |  |  |  |  |
| K665     | 8                     | 4             | 3.9                          | 5.6         | 2.5         | 158,500                        | 12           | 34             | 316                 |  |  |  |  |
| K666     | 3                     | 9             | 4.2                          | 2.1         | 5.7         | 165,000                        | 22           | 47             | 345                 |  |  |  |  |
| K667     | 15                    | 3             | 5.6                          | 10.5        | 1.9         | 163,500                        | 21           | 42             | 311                 |  |  |  |  |
| K668     | 3                     | 15            | 6.45                         | 2.1         | 9.45        | 170,500                        | 0            | 0              | 332                 |  |  |  |  |
| K669     | 5.5                   | 5.5           | 3.65                         | 3.85        | 3.5         | 188,000                        |              |                |                     |  |  |  |  |

As a further example, we have chosen three alloys of our invention having a total of 15% (within the optimum range) of metal alloying content:

Table III

| Item | Composition |      |     | Tensile Strength | Elongation | Reduction of Area |
|------|-------------|------|-----|------------------|------------|-------------------|
|      | Fe          | Cr   | Mo  |                  |            |                   |
| 1    | 5.5         | 3.5  | 6.0 | 156,200          | 22         | 50                |
| 2    | 5.0         | 7.0  | 3.0 | 152,600          | 23         | 53                |
| 3    | 5.25        | 5.25 | 4.5 | 155,200          | 23         | 43                |

In the above Table III, the alloys were tested as one half inch square bars annealed 1400° F. for one half hour and air cooled.

The result of reheating the alloys of Table III after a solution heat treatment is indicated as follows:

Table IV

| Item | Fe   | Cr   | Mo  | Rockwell "C" Hardness After Indicated Heat Treatment |                  |                  |                   |                   |
|------|------|------|-----|------------------------------------------------------|------------------|------------------|-------------------|-------------------|
|      |      |      |     | 1,500° F., 45 min. Water Quench                      | +600° F., 6 hrs. | +700° F., 6 hrs. | +700° F., 24 hrs. | +600° F., 24 hrs. |
| 1    | 5.5  | 3.5  | 6.0 | 34.5                                                 | 38.5             | -----            | -----             | 45.0              |
| 2    | 5.0  | 7.0  | 3.0 | 35.0                                                 | 36.0             | -----            | -----             | 44.5              |
| 3    | 5.25 | 5.25 | 4.5 | 36.0                                                 | 44.0             | 48.0             | -----             | -----             |

What we claim is:

1. A titanium base alloy composition having an all beta-phase structure as solution treated at a temperature of about 1200° or 1500° F., followed by air cooling, which structure is wholly stable at room temperature, and which alloy composition consists of oxygen in the amount up to about .20% maximum, nitrogen in the

8% iron, and the remainder titanium with incidental impurities; the total metal alloying content of molybdenum, chromium and iron being highly critical within the range of about 11 to 20%.

25 2. A titanium base alloy as defined in claim 1 wherein the total metal alloying content is within a range of about 13 to 16%.

30 3. A titanium alloy composition having an all beta-phase structure as solution treated at a temperature within a range of 1200° to 1500° F., followed by air cooling, which structure is wholly stable at room temperature, and which alloy composition consists of oxygen in the amount up to about .20% maximum, nitrogen in the amount up to about 11% maximum, about 2.5 to 6.5% each of molybdenum and chromium, about 3.5 to 6% iron, the molybdenum plus chromium plus iron content being within a highly critical range of above about 11% and below about 20%, and the remainder titanium with incidental impurities.

35 40 4. An improved titanium base alloy as defined in claim 11 wherein the total molybdenum plus chromium plus iron content is within a range of about 13 to 16%.

45 References Cited in the file of this patent

UNITED STATES PATENTS

|           |                     |               |
|-----------|---------------------|---------------|
| 2,554,031 | Jaffee et al. ----- | May 22, 1951  |
| 2,575,962 | Jaffee et al. ----- | Nov. 20, 1951 |
| 2,588,007 | Jaffee -----        | Mar. 4, 1952  |
| 2,640,773 | Pitler -----        | June 2, 1953  |

FOREIGN PATENTS

|         |               |               |
|---------|---------------|---------------|
| 718,822 | Germany ----- | Mar. 24, 1942 |
|---------|---------------|---------------|

55 OTHER REFERENCES

"Product Engineering," November 1949. Page 150.  
Journal of Metals, March 1950. Pages 539-552.  
Industrial and Engineering Chemistry, February 1950.

60 Pages 222-226.